

# UNITED STATES PATENT OFFICE.

ROY LINDEN HILL, OF TAMAQUA, PENNSYLVANIA, ASSIGNOR TO ATLAS POWDER COMPANY, OF WILMINGTON, DELAWARE, A CORPORATION OF DELAWARE.

## EXPLOSIVE MIXTURE.

1,360,399.

Specification of Letters Patent. Patented Nov. 30, 1920.

No Drawing. Application filed August 30, 1918, Serial No. 252,028. Renewed October 8, 1920. Serial No. 415,774.

To all whom it may concern:

Be it known that I, ROY LINDEN HILL, a citizen of the United States, residing at Tamaqua, in the county of Schuylkill and State of Pennsylvania, have invented certain new and useful Improvements in Explosive Mixtures, of which the following is a specification.

My invention relates to a non-freezing, high strength explosive mixture. I have discovered that a particularly efficient mixture of very high explosive strength is that containing ammonium perchlorate and nitro starch in the correct proportions for perfect combustion.

I have also found that other proportions of ammonium perchlorate and nitro-starch may be used, and that many other substances may be added, either to decrease the explosive strength of the mixture where a lower strength explosive is desired, to obtain desired densities, or to obtain varied rates of detonation, or varied sensitiveness, or for other purposes.

It should be understood that I do not claim as my invention mixtures of ammonium perchlorate with substances other than nitro-starch, but that I do claim broadly mixtures of ammonium perchlorate and nitro-starch in varying proportions, as the essential constituents of my new explosive mixtures, and I propose to combine with my essential ingredients varying proportions of other substances, added to produce explosive mixtures characteristically different, substantially as described above.

The foregoing several subsidiary features may or may not be employed and therefore this application will be devoted to the patenting of the compound consisting of ammonium perchlorate and nitro-starch irrespective of what other subsidiary features may be resorted to in conjunction therewith, these subsidiary features being made the subject of a separate application of even date herewith, it being apparent that the

mixture of ammonium perchlorate and nitro-starch is of utility and advantage whether any other ingredients are incorporated or not. One composition that I have found to give excellent results consists of the following ingredients combined in substantially the proportions stated, viz:

|                                                                                                               |           |    |
|---------------------------------------------------------------------------------------------------------------|-----------|----|
| Ammonium perchlorate (water proofed or otherwise)-----                                                        | 45 to 55% | 55 |
| Nitro-starch -----                                                                                            | 35 to 45% |    |
| Compounds or mixtures of compounds containing a metal or metals which will readily combine with chlorin ----- | 0 to 10%  | 60 |
| An oil or other liquid to prevent dustiness -----                                                             | 0 to 5%   |    |

For the compound or mixture of compounds containing a metal or metals which will readily combine with chlorin I have used such substances as sodium nitrate and manganese dioxide.

Having thus clearly described my invention, what I claim to be new and desire to protect by Letters Patent is:

1. An explosive mixture consisting essentially of ammonium perchlorate and nitro-starch.
2. An explosive mixture consisting of the following ingredients combined in substantially the proportions stated

|                           |           |    |
|---------------------------|-----------|----|
| Ammonium perchlorate----- | 45 to 55% |    |
| Nitro-starch -----        | 35 to 45% | 80 |

3. The new and useful composition of matter, suitable for use as an explosive, consisting of ammonium perchlorate and nitro-starch in such proportions that practically complete combustion will result on explosion.

In testimony whereof I affix my signature in the presence of two witnesses.

ROY LINDEN HILL.

Witnesses:

R. M. COOK,  
N. T. STRANE.